

Oct. 29, 1940.

M. N. NICKOWITZ

2,219,697

ARTICLE OF MANUFACTURE

Filed Sept. 21, 1939



Inventor  
Max Nathan Nickowitz

By A. F. Miller

Attorney

## UNITED STATES PATENT OFFICE

2,219,697

## ARTICLE OF MANUFACTURE

Max Nathan Nickowitz, Bridgeport, Conn., assignor to E. I. du Pont de Nemours & Company, Wilmington, Del., a corporation of Delaware

Application September 21, 1939, Serial No. 295,961

2 Claims. (Cl. 36—44)

This invention relates to insoles for shoes.

This application is a continuation in part of my application Serial Number 168,707 filed October 13, 1937.

5 A process of manufacturing shoes in which the sole is cemented to the insole (there being no midsole) has in recent times attained great commercial importance. Efforts to use leather substitute insoles in such a process have heretofore 10 been commercially unsuccessful. The stocks or sheet materials proposed for use in lieu of leather in such manufacture have had a number of prohibitive disadvantages.

A very desirable insole (or sole support) for 15 this type of shoe can be manufactured by splicing or cementing a flexible ball portion to stiff toe and/or heel portions having suitable characteristics. Heel and toe portions that are tough and stiff prevent buckling during the lasting operation and prevent the pulling through of the 20 lasting and heel attaching nails.

This invention had for an object the preparation of an improved insole and insole material. Other objects were to devise an insole of improved 25 characteristics, to prepare an insole of materials that are cheaper and more readily available than leather, and to prepare an insole which could be used in the manufacture of shoes by cementing (for example, Compo) processes. 30 Still another object was to produce an insole which could be used in the manufacture of shoes by either a cementing or sewing process. A general advance in the art and other objects which will appear hereinafter were also contemplated.

35 It has now been found that an insole having the aforementioned desirable properties and accomplishing the aforementioned objects may be prepared by laminating a rigid fiber board with a porous absorbent paper and splicing toe and 40 heel portions of such laminated material to a flexible ball portion.

My invention in its preferred form is illustrated in the accompanying drawing in which:

Figure 1 is a bottom view representing somewhat 45 diagrammatically one form of the insole of this invention.

Figure 2 is a sectional view of the insole of Figure 1, the section being along the line 2—2 of Figure 1.

50 Figure 3 illustrates one kind of blank from which the insole represented in Figure 1 might be cut.

Figure 4 is an enlarged sectional view corresponding to the lower splice portion of Figure 2 and illustrates a modified form of the invention.

55 Figure 5, similarly to Figure 4, illustrates still another form of splice, and

Figure 6 is an enlarged sectional view corresponding to the upper end of Figure 2 and illus-

trates the position of the insole in an assembled shoe.

Similar characters refer to similar parts throughout the drawing.

Referring to the drawing, the insole illustrated in Figure 1 comprises a ball portion 1 of flexible material such as low grade leather but preferably of porous absorptive material such as the latex saturated paper referred to hereinafter, a toe portion 2 of stiff, tough material capable of resisting the pulling through of nails used in the lasting operation and a unitary portion constituting the shank 3 and heel 4 composed of the same material as the toe portion 2.

As will be clear from the sectional view in Figure 2, the ball portion illustrated consists of a single thickness (laminated material can be used if desired) of material. The toe portion is laminated and comprises a layer 225 of tough stiff fiber board cemented by a layer of cement 227 to a porous, bibulous layer 226 of paper or the like which, as shown in the drawing is substantially thinner than the fiber board layer. The laminated toe portion is secured to the ball portion by a layer of cement 228.

The shank-heel portion is similar to the toe portion and comprises a tough fiber board lamina 25 secured by a cement (usually rubber cement) layer 27 to the bibulous layer 26. The rear (shank-heel) portion of the insole is secured to the ball portion by a layer of cement 28 in the same manner as the toe portion.

The end edges of tough fiber-board layers are joined to the end edges of the ball portions since it is not possible to accomplish the objects of this invention by attaching the hard layers to one side of a single sheet of the absorbent material constituting the ball portion. In such construction the hard layers when thin enough to give the substantially continuous surface desired for the present purpose would be too thin to give the required reinforcement to the soft, flexible ball portion used in the practice of this invention. The hard reinforcing layer should be as thick as possible and may practically approach the thickness of the ball portion. The absorbent layer of the toe and heel portions on the other hand should be quite thin and is desirably not more than 25% of the total thickness of the heel or toe portions. When the hard layers 25 and 225 are made the thickness of the ball portion and the paper or absorbent layer of the toe and heel portions is so thin that the surfaces of the ball portions and that of the paper toe and heel portions can be regarded as substantially continuous.

The stock from which the insole is cut is preferably manufactured in sheets. These sheets may vary in size so that one or a plurality of insoles may be cut therefrom. A blank suitable for the cutting of a single insole is illustrated in

Figure 3. The dotted line 30 indicates the outline to be followed in cutting or stamping the insole therefrom. The full and dotted parallel lines in this figure illustrate the splices, as will be clear from comparison with Figures 1 and 2. Figure 1 illustrates an insole cut from a blank large enough to yield several insoles. The full and dotted lines in Figure 1 representing the edges of the splices are shown as parallel to each other and in commercial operation they are also parallel to the edges of the blank from which they are cut. By using insoles in which the two splices have parallel edges, the blanks can be economically cut in long rows from the stock without changing the alignment of the stamping die or dies relative to the splice lines.

It is not necessary to cement the toe and/or heel-shank portions to the ball portion as illustrated in Figures 1 and 2. If desired, the attachment may be made by means of stitching, stapling or equivalent means, including various combinations of cementing, stitching and stapling. In Figure 4 one such modification is illustrated. The ball portion 41 is attached by lines 20 of stitching 49 to the shank portion which comprises laminae 45 and 46 united by a layer of cement 47. The tough fiber board layer is shown at 45.

In Figure 5 a still further modification (employing stapling) is shown. In this figure the flexible ball portion 51 is united to the shank portion by means of a single line of stapling 59 and a layer of cement 58. The layers indicated at 55, 56 and 57 correspond to the layers 25, 26 30 and 27, respectively, in Figure 2.

As previously indicated, the sole of the shoe utilizing this invention is cemented to the insole after the insole has been nailed or otherwise attached to the upper portion of the shoe. The 40 relation of the sole and insole (at the toe) is illustrated in Figure 6, wherein the insole assembly comprising a tough fiber board layer 6225 is united to a porous lamina 6226 by means 45 of a cement layer 6227. In this assembly the shoe sole 6 is united to the absorptive layer 6226 by means of a layer of cement 67. Methods of joining sole and insole are well known in the art (see for example U. S. Patent 1,967,337).

The lamination of the toe and the shank-heel stock is usually carried out before the skiving and cementing of these portions to the skived flexible ball portion. It is possible to cut the various portions of the insole to shape and there- 50 after assemble them, and to partly assemble, cut and then finish assembling, but in commercial practice a stock sheet material is prepared and shipped to the shoe manufacturer who cuts or stamps insoles of various sizes and types 55 therefrom. This has been found to be a more economical procedure.

The toe and shank-heel portions are ordinarily made up of two layers of material permanently laminated by means of suitable cement. In the 65 insole illustrated in the drawing these portions consisted of a layer of tough stiff fiber board cemented to a porous layer of paper. In some instances it may be desirable to cement an absorptive layer to both sides of the stiff layer. 70 Even more laminae may be used for special purposes.

In making the toe and shank-heel portions any stiff rigid sheet material otherwise suitable for insole construction may be used for the tough

layer. In the place of the fiber board mentioned above, other absorptive material such as paper, which has been impregnated and/or coated with a resinous material to render it stiff and rigid, may be used. The chief requirement is that the 5 stock used have sufficient rigidity and toughness to withstand the lasting operation and pulling through of the lasting and heel attaching nails. A wide range of materials are suitable for the absorptive layer. Mention may be made of sized 10 and unsized woven fabrics, woven fabrics saturated with latex, sized and unsized paper, paper saturated with binders such as glue, casein, shellac, asphalt and rubber, leather skivings, split leather and the like. The preferred material is 15 a rubber saturated paper, in which the rubber has been applied in the form of latex. Satisfactory material is also obtained by substituting rubber cement for the latex. The paper may be 20 saturated by passing it, while dry, through a bath of rubber cement or latex, squeezing out the latex and drying. The material produced according to United States Patent 1,966,458 is especially suitable. In general any porous material 25 capable of readily absorbing a layer of shoe cement and having properties otherwise suitable for insole construction may be used.

The materials mentioned for the porous layer of the toe and shank-heel portions are in general 30 suitable for the ball portion. In addition, such materials as leather, artificial leather, leather substitutes and the like may be used.

The most valuable embodiment of this invention is that in which the absorptive ball portion, 35 and preferably also the absorptive laminae at heel and toe, consists of a latex saturated paper containing rubber sufficient to confer the required strength but insufficient to prevent the sole absorbing the adhesives used in shoe making. 40 Once the sole is cemented to the shoe the internal strength is sufficient to prevent internal fiber separation when a strain is not upon the sole. For the present purpose the rubber in the latex 45 impregnated paper should not usually be above 35% or below 15% and is ordinarily about 20%. A typical latex impregnated paper suitable for the present purpose is one consisting of about 43% unbleached kraft pulp, 21% wood flour, 21% chrome leather, and 15% rubber. Another 50 example of a similar product is one having the approximate composition of 54% paper pulp, 7% wood flour, 7% asbestos, 17% chrome leather, and 15% rubber.

Any type of adhesive cement which will unite 55 the plies of the laminated portions and which will unite the resultant laminated material to the flexible ball portion, may be used. Rubber cements have been found to be especially suitable 60 for these purposes. A typical cement is given in Example I.

|         | Per cent by weight |
|---------|--------------------|
| Rubber  | 60 85              |
| Rosin   | 4                  |
| Factice | 10                 |
| Whiting | 26                 |
| Total   | 100 70             |

In attaching the sole to the insole, the standard air-drying pyroxylin cements are used. Such cements are well known to those skilled in the art and in the patent literature (see for example U. S. 75

Patent 1,959,323). Specific typical examples of such compositions are given in Examples II and III.

*Example II*

|                           | Per cent by weight |
|---------------------------|--------------------|
| Nitrocellulose            | 15                 |
| Camphor                   | 4                  |
| Ethyl alcohol (denatured) | 10                 |
| Acetone                   | 51                 |
| Ethyl acetate             | 20                 |
| <b>Total</b>              | <b>100</b>         |

*Example III*

|                   | Per cent by weight |
|-------------------|--------------------|
| Pyroxylin         | 15                 |
| Dibutyl phthalate | 2                  |
| Camphor           | 1                  |
| Ethyl alcohol     | 5                  |
| Acetone           | 77                 |
| <b>Total</b>      | <b>100</b>         |

The nitrocellulose in these compositions preferably has a viscosity of 20-30 seconds, as determined by the method outlined in the A. S. T. M. specifications D-301-31T formula A, and a nitrogen content of 12.30 to 12.50% as determined according to the A. S. T. M. specifications D-301-31T. These examples are given for purposes of illustration, and are merely representative of many pyroxylin cements suitable for use in the well known Compo processes of shoe manufacture.

As previously indicated, the character of the various parts of the insole will vary somewhat with the use to which the insole is to be put, as for example, an insole suitable for ladies' evening slippers and like uses may consist of a ball portion  $\frac{1}{8}$ " thick and weighing 4 ounces per square foot, a toe-heel portion having an absorptive layer  $\frac{1}{2}$ " thick weighing 1 ounce per square foot, and a tough, stiff fiber board layer  $\frac{1}{2}$ " thick weighing 3 ounces per square foot. Obviously the insole of footwear subject to more severe condi-

tions would require proportionately heavier and stronger construction in some or all of the above component parts.

The insole of this invention makes it possible to use paper, fiber board and like leather substitutes in the manufacture of shoes by the so-called cement processes. The conventional shoe cements will "bite in" to these insoles in the time allowed for such an operation in present commercial practice in the manufacture of cement 10 lasted shoes.

As many apparently widely different embodiments of this invention may be made without departing from the spirit and scope thereof, it is to be understood that I do not limit myself 15 to the specific embodiments thereof except as defined in the appended claims.

I claim:

1. An insole adapted to be cemented to a shoe sole which comprises a flexible porous absorptive 20 ball portion and laminated toe and heel portions comprising at least two laminae attached to the ends of said ball portion, the laminae of both said portions being separate from said ball portion, one lamina of each of said toe and heel portions 25 on the same side of the insole being a layer of stiff tough material joined at an end edge to an end edge of the ball portion whereby the surfaces of said ball portion and tough layers are substantially continuous, the other of said laminae consisting of a layer of absorbent material attached to each of the tough layers at the side of the sole 30 opposite said surfaces, said layers of absorbent material being substantially thinner than said layers of tough material. 35

2. An insole adapted to be cemented to a shoe sole which comprises a ball portion consisting of a latex impregnated paper absorptive to shoe cement, and laminated toe and heel portions joined to the end edges of the ball portion, said 40 laminated portions each comprising a layer of fiber-board having attached to one face thereof a layer of latex impregnated paper which is substantially thinner than said fiber-board layer.

MAX NATHAN NICKOWITZ.

45